

A. S. DWIGHT,  
PROCESS OF TREATING ORES TO SINTER THEM.  
APPLICATION FILED MAY 8, 1912.

1,433,351.

Patented Oct. 24, 1922.

2 SHEETS—SHEET 1.



Fig. 1.



Fig. 2.

WITNESSES

Marshall Dow  
S. Jay Teller

INVENTOR

Arthur S. Dwight  
By H. H. Bliss  
Attorney

A. S. DWIGHT.

PROCESS OF TREATING ORES TO SINTER THEM.

APPLICATION FILED MAY 8, 1912.

1,433,351.

Patented Oct. 24, 1922.

2 SHEETS—SHEET 2.



Fig. 3.



Fig. 4.



Fig. 5.

WITNESSES.

Marshalllow  
S. Jay Teller

INVENTOR

Arthur S. Dwight  
By ~~At~~ <sup>At</sup> ~~or~~ <sup>or</sup> ~~Seal~~ <sup>Seal</sup>  
attorney

## UNITED STATES PATENT OFFICE.

ARTHUR S. DWIGHT, OF NEW YORK, N. Y., ASSIGNOR TO DWIGHT & LLOYD METALLURGICAL COMPANY, OF NEW YORK, N. Y., A CORPORATION OF NEW JERSEY.

## PROCESS OF TREATING ORES TO SINTER THEM.

Original application filed December 23, 1907, Serial No. 407,860. Divided and application filed March 25, 1912, Serial No. 685,909. Divided and this application filed May 8, 1912, Serial No. 695,882.

To all whom it may concern:

Be it known that I, ARTHUR S. DWIGHT, a citizen of the United States, residing at New York, in the county of New York and State of New York, have invented certain new and useful Improvements in Processes of Treating Ores to Sinter Them, of which the following is a specification, reference being had therein to the accompanying drawings.

10 My invention relates to the art of treating ores for the purpose of sintering them, especially such ores as contain or have mixed with them a readily combustible element or substance and are of such nature that combustion may be carried on therein after an initial igniting of the mass has been effected; and which may, by reason of the said combustion carried on while the contiguous particles of the mass are maintained as to each 15 other in a state of relative quiescence, be sintered or have the particles thereof aggregated into masses which are well suited for subsequent treatment in blast furnaces. I may mention as one example of an ore such 20 as the process and apparatus herein to be described are adapted to treat, a sulfid ore in which the combustible constituent, sulfur, is in sufficient quantity to permit the ore to be readily ignited and to burn if supplied 25 with air or other supporter of combustion; and as another example of the material to be treated, I may mention a mixture of pulverized or finely crushed ore and pulverized coal or other form of carbon.

30 The invention herein presented and claimed relates particularly to the means employed for effecting the initial ignition of the ore. Such means are capable of combination with any of numerous sorts of 35 mechanisms for supporting and for carrying the ore during and after treatment, and in respect to said supporting and carrying mechanisms the present invention is not limited.

40 For the purpose of illustrating how the invention may be practically carried into effect, I have represented in the accompanying drawings, the mechanism for supplying and transporting the ore, and finally delivering it in sintered masses, which is shown, described, and claimed in my application for patent filed December 23, 1907, original Serial Number 407,860 on which application has issued Patent #1,027,110 dated

May 21, 1912. This application is a division of my application 685,909 filed March 25, 1912, which is itself a division of my aforesaid application filed December 23, 1907, No. 407,860, in which earlier divisional application are presented claims for the mechanism illustrated and described in this application in so far as it relates to the means shown for igniting the ore at its surface, in an ore sintering or agglomerating apparatus. I therefore herein make no claim to such apparatus.

55 Figure 1 is a side elevation of an ore sintering machine such as just referred to and with which the improvements herein presented and claimed are adapted to be used.

60 Fig. 2 is a cross sectional view of part of the apparatus illustrating the igniters.

65 Fig. 3 is a cross section showing one of the pallets or ore carrying elements and part of the suction box.

70 Fig. 4 is a longitudinal sectional view of a part of the apparatus taken on the line IV-IV of Fig. 5.

75 Fig. 5 is a top plan view.

80 For the purposes hereof it is sufficient to note that, in the drawings, A represents an air suction box, over or across the open end of which travel the ore-supporting cars or pallets B, these constituting individual elements of a carrier for the ore. Each of 85 these elements carries one or more grate sections C, suitably supported, and is mounted upon wheels D adapted to travel upon tracks or guides, shown at F, F', F'.

90 K indicates a hopper or feeder which is supplied with ore, initially, and from which it is delivered in charges or in a stream to the cars or pallets B, so that each element supports a thin pervious bed or layer of the ore.

95 After the ore has been placed upon its support or carrier, it is ignited at its open or exposed surface by the temporary application thereto of flame or burning products which are so regulated and controlled as to 100 subject a relatively wide area of the surface of the ore bed to a simultaneous treatment for ignition. After this temporary application of the flame or burning products, which is maintained sufficiently long for perfect ignition, the ore is subjected to a more or less 105 extended and continuous action of the air currents which are induced to pass through

the body of ore by the air moving mechanism U connected with the air box or chamber A. In operating with the mechanism illustrated in the drawing, the ore carrier, formed of the units designated B, is slowly moved across the open end of the air chamber A, the length of such open end, and the speed at which the carrier moves determining the length of time when the ore is subjected to the action of the air currents passing through the ore body, during which time such internal combustion takes place within the ore mass as to cause the desired sintering thereof, and the desulfurizing, when a sulfid ore is being treated. At the end of the track section F, which is the section adjacent to the open end of the wind box or air chamber A, and which, as shown, preferably extends some distance beyond the end of the wind box, the ore carriers pass to the downwardly curved track section or guide, F', with which the wheels of the pallets or individual ore carriers engage and by which their course is directed. From this part of the guideway the pallets or cars move to the inclined and returning part of the track, F<sup>2</sup>, along which they travel in inverted position. At H there are lifting and power transmitting wheels, adapted to engage with the pallets or cars and carry them upward to the track section F, and then by a pushing action impart forward travel to them during their next cycle. The wheels H are rotated by the belt T connected with their shaft. At U there is an air forcing apparatus, here shown as a suction fan, connected by a trunk or duct J, with the air box A, and adapted to exhaust the air from the latter, causing currents of air to pass downward through the ore on the pallets or cars, as indicated by the arrows in Fig. 1.

The means which are herein shown for igniting the ore are adapted for burning gasolene, petroleum, or other similar combustible fluid, and preferably comprise a pair of spray burners I', so arranged that the flames and burning products issuing therefrom, are applied to and caused to pass over and across the upper exposed surface of the mass of ore to be treated. The burners I' are preferably disposed diametrically opposite each other as represented in Fig. 2. The burners are supplied through a pipe, I, connected with any suitable source of supply and are provided with the regulating valves i, i. It will be apparent that by apparatus such as I have described a broad and intense flame is caused to be passed over and across a sufficiently wide area of the ore at one and the same instant of time to insure perfect ignition, and that the flame is drawn into intimate contact with the surface of the ore, and somewhat into the body thereof, by the suction apparatus connected with the air box A. In these respects the

igniter herein described and illustrated differs from igniting apparatus which I have illustrated in earlier patents of mine, for instance, in Patent 916,391 of March 23, 1909, wherein I show an igniter consisting of a perforated gas pipe extending across the apparatus supporting the bed of ore and arranged to direct small open jets of gas against the surface of the ore along a narrow line.

The present apparatus not only possesses the advantage of subjecting a comparatively large area of the exposed body of ore to the igniting flame at one and the same instance, but is adapted to be used in localities where gas is not easily obtainable and where, therefore, an apparatus of the sort illustrated in my aforesaid patent could not be used to advantage.

By means of the regulating valves i, the volume and intensity of the flames issuing from the burners can be varied to suit the different conditions met with in treating ores; and moreover by means thereof the flames can be temporarily entirely cut off or so reduced as to have no igniting effect upon the ore, and then again increased so as to project across a fresh surface of the ore to be ignited, this latter method of manipulation being desirable where the ore is of such character as to be quickly ignited, and hence requiring but a relatively very short application of the igniting flames.

It will be seen that in the apparatus shown there is relative movement between the body of the ore and the igniting burners, as well as movement of the flames that issue from the burners across and over the body of the ore.

I have not in the drawings illustrated in detail the construction of the spray burners I', as they may be of any well known kind adapted to the use described.

In using the apparatus shown the ore carrier is slowly moved by the wheels H, and the elements thereof are filled from the hopper K, each receiving a relatively thin layer which is uniformly spread upon the grate C. After the ore has been properly deposited it is ignited at its upper surface by the means already described, and, after being thoroughly ignited the play of the hot igniting particles upon the surface of the ore is discontinued, either by reason of relative separating motion between the ignited ore mass and burners; or by movement of the flaming particles and hot products of combustion over, across, and relative to the ore, as by the intermittent shutting off and admitting of the fuel supply to the burners. The ore being once thoroughly ignited at its surface, a uniform combustion transversely through the ore mass is caused to take place by currents of air which are induced, by the air moving apparatus U, to

pass through the bed of ore, the combustion, which is carried on while the contiguous particles of the mass are in a state of relative quiescence, being sufficiently active to insure sintering or agglomerating of the particles of ore. The apparatus is so operated that a sintering of the entire mass of ore supported by any pallet or carrying element is completed at about the time or shortly before it arrives at the place of discharge. The manner of breaking up the sintered ore masses and discharging them, and causing the sintered cakes to separate themselves from the grates or perforated supports as the pallets are inverted, need not be described in this case, as these operations do not form a part of the invention to which the present case has particular reference.

It will be seen that, in carrying out this process in the manner herein illustrated and described, the ore material, from the time it is delivered to the pallets until it is finally discharged therefrom as a sintered product, is maintained in a quiescent state, there being no agitation of its particles during this period. The ore-holding devices shown receive the ore in the way illustrated in a relatively shallow layer or stratum and it passes from the place of initial feeding to the place of sinter delivery without contacting with any devices that would act to stir, disturb or agitate it. The air guiding mechanism is such that the air moves from the top of the stratum through it toward the bottom to support internal combustion, and this method of applying and directing the air is adopted because the air passing through in this way does not agitate the particles in relation to each other and they are permitted to remain in quiescence.

I do not in this case claim the mechanism for supporting and conveying the ore and for causing air currents to pass through the ore while being supported and conveyed which is illustrated and described in this application, as such apparatus is claimed in my aforesaid Patent #1,027,110. The said mechanism in so far as it is a conveying apparatus capable of use for other purposes than in the roasting, sintering and similar treatment of ore, is also claimed by me in my application filed April 30, 1910, Serial No. 558,621 on which has issued Patent #1,027,111 dated May 21, 1912.

What I claim is:—

1. In the art of sintering ore, the herein described process which consists in forming a thin pervious bed of ore containing a combustible constituent, igniting the ore at an exposed surface thereof by a broad mass of highly heated products of combustion applied across a relatively wide area of the ore surface at one and the same period of time and continuing the combustion thus started

while the contiguous particles of the mass are maintained in a condition of relative quiescence.

2. In the art of sintering ore, the herein described process which consists in forming a thin pervious bed of ore containing a combustible constituent, igniting the ore at an exposed surface thereof by a broad mass of highly heated products of combustion applied across a relatively wide area of the ore surface, drawing the said igniting heated products of combustion into intimate contact with the ore by means of air currents passing through the ore mass and continuing the combustion thus started while the contiguous particles of the mass are maintained in a condition of relative quiescence.

3. In the art of sintering ore, the herein described process which consists in forming a thin bed of ore containing a combustible constituent, igniting the ore at an exposed surface by flaming particles issuing from a burner and causing the said flaming particles to be projected from the burner and to spread over and across an exposed surface of the ore and continuing the combustion thus started while the contiguous particles of the mass are maintained in a condition of relative quiescence.

4. In the art of sintering ore, the herein described process which consists in forming a thin pervious bed of ore containing a combustible constituent, igniting the ore at an exposed surface thereof by flaming particles issuing from a burner, causing the said flaming particles to be projected from the burner and to spread over and across an exposed surface of the ore, discontinuing the play of the igniting flaming particles upon the ore and then completing the sintering by internal combustion within the ore mass while the particles thereof are maintained in a state of relative quiescence.

5. In the art of sintering ore, the herein described process which consists in forming a thin pervious bed of ore containing a combustible constituent, igniting the ore at the exposed upper surface thereof by flaming particles of burning liquid hydrocarbon drawn into intimate engagement with the ore by air currents passing downwardly through the said bed of ore, the combustion thus started being continued through the mass while the contiguous particles thereof are maintained in a state of relative quiescence.

6. In the art of sintering ore, the herein described process which consists in forming a thin pervious bed of ore containing a combustible constituent, igniting the ore at an exposed surface thereof by flaming particles of burning liquid hydrocarbon which are temporarily applied to a relatively wide area of the exposed surface of the ore at one and the same period of time, discontinuing

the play of the igniting flaming particles upon the ore after thorough surface ignition has taken place, and continuing the sintering by internal combustion in the ore mass induced by air currents passing through the bed of ore while the particles thereof are maintained in a state of relative quiescence.

7. In the treatment of ore or other material containing a combustible component, the process of subjecting a charge of the material to the traverse of gases through the charge from top downward, projecting from fixed points above the charge ignition fuel across the surface of the charge in paths substantially parallel to said surface and under a head to overcome any material deflection from said paths by the currents traversing the charge, and supplying combustion-supporting gases to said ignition fuel.

8. In the art of sintering or agglomer-

ating fine ore containing a combustible constituent, the process herein described which consists in disposing the ore in a relatively thin layer permeable to gases, moving the ore layer along a prescribed path, projecting across the exposed surface of the layer, from the side edges thereof and substantially at right angles to the direction of movement of the ore layer, burning or flaming fuel to ignite the ore at its surface, drawing air through the ore layer to maintain internal combustion therein, and continuing such internal combustion after the ore layer has been moved past the place of ignition thereof.

In testimony whereof I affix my signature, in presence of two witnesses.

ARTHUR S. DWIGHT.

Witnesses:

ROBERT C. CONLY,  
LOUIS H. HYDE.

## DISCLAIMER

1,433,351.—*Arthur S. Dwight*, New York, N. Y. PROCESS OF TREATING ORES TO SINTER THEM. Patent dated October 24, 1922. Disclaimer filed October 21, 1931, by the assignee, *Dwight & Lloyd Sintering Company, Inc.*

Hereby enters this disclaimer to claims 3, 4, 5, and 7 of said Letters Patent, which are in the following words, to-wit:

“3. In the art of sintering ore, the herein described process which consists in forming a thin bed of ore containing a combustible constituent, igniting the ore at an exposed surface by flaming particles issuing from a burner and causing the said flaming particles to be projected from the burner and to spread over and across an exposed surface of the ore and continuing the combustion thus started while the contiguous particles of the mass are maintained in a condition of relative quiescence.

“4. In the art of sintering ore, the herein described process which consists in forming a thin pervious bed of ore containing a combustible constituent, igniting the ore at an exposed surface thereof by flaming particles issuing from a burner, causing the said flaming particles to be projected from the burner and to spread over and across an exposed surface of the ore, discontinuing the play of the igniting flaming particles upon the ore and then completing the sintering by internal combustion within the ore mass while the particles thereof are maintained in a state of relative quiescence.

“5. In the art of sintering ore, the herein described process which consists in forming a thin pervious bed of ore containing a combustible constituent, igniting the ore at the exposed upper surface thereof by flaming particles of burning liquid hydrocarbon drawn into intimate engagement with the ore by air currents passing downwardly through the said bed of ore, the combustion thus started being continued through the mass while the contiguous particles thereof are maintained in a state of relative quiescence.”

“7. In the treatment of ore or other material containing a combustible component, the process of subjecting a charge of the material to the traverse of gases through the charge from top downward, projecting from fixed points above the charge ignition fuel across the surface of the charge in paths substantially parallel to said surface and under a head to overcome any material deflection from said paths by the currents traversing the charge, and supplying combustion-supporting gases to said ignition fuel.”

[Official Gazette November 17, 1931.]